

## UNITED STATES PATENT OFFICE

2,538,417

## INDIUM PLATING

David Frederick Green and John Ernest Salmon,  
London, England, assignors to Vandervell  
Products Limited, London, England

No Drawing. Application November 7, 1945, Se-  
rial No. 627,278. In Great Britain January 2,  
1945

6 Claims. (Cl. 204—45)

1

This invention relates to indium plating particularly in its relation to electroplating bearing surfaces.

In the specification of our U. S. application Ser. No. 604,524, now Patent No. 2,497,988, dated February 21, 1950, a stable electrolytic bath is described which consists of an indium salt, alkali metal cyanide and hydroxide and dextrose or other suitable saccharide. While other indium salts may be used the use of the chloride is preferred. Our research has established that it is not necessary to use a saccharide as laid down in our prior specification above referred to, but that other materials such as certain polyhydric alcohols can be used and sorbitol has been found particularly suitable. The sorbitol can be substituted for dextrose in the solutions described in our prior specifications in similar concentrations and solutions so prepared can be used to prepare a solid residue which can be stored and transported conveniently and then used to reconstitute a plating solution merely by dissolving in water and adjusting the free alkali metal cyanide and hydroxide contents to the desired concentrations.

Alternatively, if desired, sufficient alkali metal cyanide and hydroxide can be mixed with the solid so that when dissolved in water it will yield a solution containing the desired concentrations of free alkali metal cyanide and hydroxide. The amount of cyanide and hydroxide required can easily be determined by dissolving a small portion of each batch in the appropriate quantity of water and analysing the solution.

Our invention may be said to consist of:

An electrolytic bath for use in electroplating with indium according to which sufficient alkali metal hydroxide is added to an electrolytic bath consisting of an indium salt, alkali metal cyanide and sorbitol or equivalent polyhydric alcohol to provide a stable solution.

The invention further comprises a process of electroplating with indium wherein such an electrolytic bath is used.

Suitable hydroxides for use in the process are sodium or potassium hydroxide, and the indium salt employed is preferably indium chloride.

One specific electrolytic bath for use in plating metals with indium, according to our invention, consists of a stable composition of indium, potassium cyanide, potassium hydroxide and sorbitol.

According to one method of preparing such an electrolytic bath comprising indium-potassium cyanide-potassium hydroxide and sorbitol the indium metal is first dissolved in an excess of concentrated hydrochloric acid and the solution evap-

2

orated until crystallisation of indium chloride occurs, and the crystallised indium chloride is then dissolved in distilled water, a second solution of potassium-cyanide and sorbitol in water and a third solution of potassium-hydroxide in water are then prepared, the first solution is then added to the second solution drop by drop accompanied by constant stirring and the third solution is then added. The quantities of the materials used being selected to obtain a stable solution. An example of these quantities which has proved satisfactory is as follows:

Indium metal, 30 grammes  
15 Potassium-cyanide, 100 grammes or approxi-  
mately 2 moles  
Sorbitol, 30 grammes  
Potassium hydroxide, 120 grammes or approxi-  
mately 2 moles

20 to make 1 litre of solution.

We claim:

1. A solid soluble mixture adapted to be dis-  
solved in water to produce an electrolytic indium  
25 plating bath which comprises indium, sorbitol,  
alkali metal hydroxide and alkali metal cyanide  
in or about the following proportions: 30  
grammes of indium as indium trichloride, 2 moles  
of alkali metal cyanide, 30 grammes of sorbitol  
and approximately 2 moles of an alkali metal hy-  
droxide.

2. A solid soluble mixture adapted to be dis-  
solved in water to produce an electrolytic indium  
35 plating bath which comprises indium, sorbitol,  
potassium hydroxide and potassium cyanide in or  
about the following proportions; 30 grammes of  
indium as indium trichloride, 30 grammes of sor-  
bitol, 100 grammes of potassium cyanide and 120  
grammes of potassium hydroxide.

3. A solid soluble mixture adapted to be dis-  
40 solved in water to produce an electrolytic indium  
plating bath which comprises indium, sorbitol,  
sodium hydroxide and sodium cyanide in or about  
the following proportions: 30 grammes of indium  
45 as indium trichloride, 30 grammes of sorbitol,  
2 moles of sodium hydroxide and 2 moles of sodium  
cyanide.

4. A method of making a water soluble mixture  
for use in preparing an indium electroplating  
50 bath according to which 30 grammes of indium  
as indium trichloride is added to a solution con-  
taining approximately 2 moles of alkali metal  
cyanide and 30 grammes of sorbitol and approxi-  
55 mately 2 moles of an alkali metal hydroxide in  
which the indium solution is added to a mixture  
of the sorbitol and cyanide accompanied by agita-

tion and subsequently the hydroxide is added and the solution is evaporated to dryness to leave a residue soluble in water.

5. A method of making a water soluble mixture for use in preparing an indium electroplating bath according to which 30 grammes of indium as indium trichloride is added to a solution containing approximately 100 grammes of potassium cyanide and 30 grammes of sorbitol and approximately 120 grammes of potassium hydroxide in which the indium solution is added to a mixture of the sorbitol and cyanide accompanied by agitation and subsequently the hydroxide is added and the solution is evaporated to dryness to leave a residue soluble in water.

6. A method of making a water soluble mixture for use in preparing an indium electroplating bath according to which 30 grammes of indium as indium trichloride is added to a solution containing approximately 2 moles of sodium cyanide and 30 grammes of sorbitol and approximately 2 moles of sodium hydroxide in which the indium solution is added to a mixture of the sorbitol and cyanide accompanied by agitation and subsequently the hydroxide is added and the solution

is evaporated to dryness to leave a residue soluble in water.

DAVID FREDERICK GREEN.  
JOHN ERNEST SALMON.

#### REFERENCES CITED

The following references are of record in the file of this patent:

#### UNITED STATES PATENTS

|    | Number    | Name          | Date          |
|----|-----------|---------------|---------------|
| 10 | 694,658   | Meurant       | Mar. 4, 1902  |
|    | 1,849,293 | Gray          | Mar. 15, 1932 |
|    | 1,965,251 | Murray et al. | July 3, 1934  |
| 15 | 2,423,624 | Smart         | July 8, 1947  |
|    | 2,458,839 | Dyer et al.   | Jan. 11, 1949 |

#### FOREIGN PATENTS

|    | Number  | Country       | Date    |
|----|---------|---------------|---------|
| 20 | 573,848 | Great Britain | of 1945 |

#### OTHER REFERENCES

- Iron Age, Dec. 19, 1940, pp. 35-38.  
Transactions of Electrochemical Society, vol. 25 65, pp. 377-383 (1934).